

# UNITED STATES PATENT OFFICE.

WILHELM THEODOR UNGE, OF STOCKHOLM, SWEDEN.

## COMPOSITION FOR FUSES AND PROCESS OF MAKING SAME.

No. 806,025.

Specification of Letters Patent.

Patented Nov. 28, 1905.

Application filed October 2, 1903. Serial No. 176,486.

*To all whom it may concern.*

Be it known that I, WILHELM THEODOR UNGE, a subject of the King of Sweden and Norway, residing in Stockholm, Sweden, have invented an Improved Slow-Combustion Composition for Fuses, Air-Torpedoes, or the Like, of which the following is a specification.

Slowly-burning compositions which generate gas on being ignited are used for many purposes. In safety-fuses, fuses for projectiles, &c., such a composition is used as the agent for effecting the ignition of a bursting charge or the like after the lapse of a predetermined time. In rockets, air-torpedoes, and the like the composition is used to provide propelling power. As a lighting agent such a composition is used in torches and the like. Such compositions are generally manufactured by pulverizing and mixing certain materials, the mixture being then compressed, so as to render it coherent and compact to such a degree that after the composition has been ignited the fire cannot penetrate into the mass, but the combustion proceeds continuously from the ignited surface. Compositions manufactured in the above manner, however, have the property of decreasing in volume during storage, even if the pulverized materials of which they are composed have been completely dry. If the latter contain any moisture, a greater shrinking of the mass during storage takes place. Such compositions also lack elasticity and are very brittle. They also are affected by damp, and from the fact of their expanding less than metal with increase of temperature it may happen that when the composition is inclosed in a metallic chamber—as, for instance, in so-called "time-fuses" for projectiles, air-torpedoes, &c.—the walls of the chamber separate from the composition when the temperature increases. For these reasons cracks are liable to be formed throughout the mass of the composition, so that when ignited the fire spreads in cracks and interstices and an explosion of the composition may occur. If such a composition is used in time-fuses, part of or the whole of the composition forming the fuse may take fire at once and cause a premature explosion of the charge ignited by the fuse. Further,

such a composition being hygroscopic the rate of combustion will vary, depending on the conditions of storage.

The object of this invention is to obviate these defects. This is effected by imparting to the particles of the composition an increased mobility among themselves by greasing them with a non-volatile oil, thus increasing their elasticity and decreasing their hygroscopic properties. As a result, the particles after compression tend to move from each other in consequence of their increased elasticity, so that the composition in case of being compressed in a chamber always tends to swell and keep the chamber full. Instead of greasing the particles with a non-volatile oil a non-volatile grease or fat or some other non-volatile greasing material, or a mixture thereof, may be used, if desired.

The composition may consist of finely-divided common black gunpowder or the materials in rocket compositions, such as carbon, sulfur, and saltpeter. It is found that a proportion of the greasing ingredient, which may be fine olive-oil, of 0.001 to 0.003 of the total weight of the composition has proved sufficient for obtaining the result aimed at; but the proportion may vary according to the circumstances.

The introduction of the greasing material into the composition may be effected in any suitable manner, either before or after the compression. Before the compression the greasing material may, for instance, be mixed mechanically with a small portion of the powder of the composition, and this portion is then afterward thoroughly incorporated with the remaining portion of the powder. After the compression the composition may be immersed in or enveloped by the greasing material and be left there until the necessary absorption has taken place.

I claim as my invention—

1. A slow-burning composition for fuses and the like, composed of compressed pulverous combustion material, having its particles greased throughout its mass with a non-volatile greasing material in about the proportions set forth, whereby the combination is rendered non-shrinking, expansive, elastic, and its hygroscopic tendency is reduced.

2. The herein-described process of producing an elastic, expansive, and non-hygroscopic combustion material for fuses or the like, consisting of incorporating with the  
5 loose fuse material a non-volatile greasing material in about the proportions set forth and then compressing the mass.

In testimony whereof I have signed my name to this specification in the presence of two subscribing witnesses.

WILHELM THEODOR UNGE.

Witnesses:

A. HELJESTRAND,

S. SOMMAR.